

Dec. 3, 1957

R. H. BECK

**2,815,307**

## PROCESSES FOR COATING AND DRYING PHOTOGRAPHIC LAYERS

Filed Aug. 20, 1953

2 Sheets-Sheet 1



FIG. 1

INVENTOR  
**ROBERT HAUN BECK**

BY Lynn Barrett Morris

ATTORNEY

Dec. 3, 1957

R. H. BECK

2,815,307

## PROCESSES FOR COATING AND DRYING PHOTOGRAPHIC LAYERS

Filed Aug. 20, 1953

2 Sheets-Sheet 2



FIG.2.



ROBERT HAUN BECK

ROBERT HAUN BECK

BY Lynn Barrett Morris

ATTORNEY

1

2,815,307

**PROCESSES FOR COATING AND DRYING  
PHOTOGRAPHIC LAYERS**

Robert Haun Beck, Fair Haven, N. J., assignor to E. I. du Pont de Nemours and Company, Wilmington, Del., a corporation of Delaware

Application August 20, 1953, Serial No. 375,404

9 Claims. (Cl. 154—102)

This invention relates to photography and more particularly to a process and apparatus for coating viscous solutions as layers in photographic elements and drying such layers. More particularly it relates to a process and apparatus for coating and drying viscous aqueous silver halide dispersions in water-permeable colloids. Still more particularly it relates to such a process and apparatus wherein highly reduced pressures are utilized. In an important aspect, the invention relates to a process and apparatus for coating and drying viscous aqueous silver halide dispersions in gelatin at highly reduced pressures.

Photographic films and paper are usually made on a large commercial scale by coating continuous rolls of flexible film base in wide widths, e. g., 36 to 48 inches, with an aqueous dispersion of silver halides in a water-permeable colloid, chilling and setting the liquid emulsion and drying the emulsion layer in a convection type dryer wherein the wet bulb temperature of the air is lower than the melting point of the set emulsion. Two common methods of coating photographic layers are: (1) skim coating in which the web is passed around a coating roll disposed in a coating pan so that the web contacts the liquid emulsion and picks up a thin layer and (2) air jet coating in which emulsion is applied by method (1) and then a thin jet of air is directed against the coating in order to control the amount (thickness) of emulsion adhering to the web. The photographic layer can also be applied by dip coating, by applicator rolls, or from a suitable extrusion hopper. The air jet method has the advantage that aqueous emulsions of higher solids content can be used.

In the procedures described above, setting of the aqueous emulsion layer is accomplished by passing the coated web through a zone in which the wet bulb temperature is below the melting point of the emulsion wherein it sets or gels to a semi-solid condition.

Drying of the webs coated by the foregoing methods is usually done by festooning the web over the moving bars of a festoon dryer. The air velocities and drying conditions in such a dryer are generally moderate and drying times of 30 to 90 minutes are required, depending upon the coating weight of the layer. Spiral chamber dryers and tenter frame dryers have been used and are quite satisfactory but they require rather expensive and large equipment.

In the processes and apparatus just described, the aqueous silver halide colloid dispersions are relatively dilute, having solids contents of about 10% to about 20%. The large amount of water in such dispersions necessitates long drying times and large size apparatus. The drying rate is limited by the air velocities used and by the capacity of the air conditioning equipment required to maintain the wet bulb temperature below the melting point of the emulsion. Under the best of conditions these prior art procedures require from 5 to 10 minutes in order to complete the drying of a section of photographic film. Similar problems are encountered in the coating of photographic paper.

2

An object of this invention is to provide an improved process for coating and drying photographic webs, e. g., films and papers. Another object is to provide a more rapid method of coating and drying photographic films and papers. A further object is to provide a process of coating films and papers with photographic emulsions of high solids content. Yet another object is to provide such a process which can be readily controlled. A still further object is to provide such a process which can be carried out on a continuous basis and will produce relatively thin, smooth, uniform coatings.

Another object of the invention is to provide improved apparatus for the coating and drying of concentrated aqueous silver halide colloid dispersions. Yet another object is to provide such apparatus which is simple to construct and easy to maintain under continuous operating conditions. A further object is to provide such an apparatus which requires a minimum of space and moving parts. Still other objects will be apparent from the following description of the invention.

The above and other objects are attained, and a commercially practical process of coating and drying a viscous aqueous solution provided by the present invention, which comprises extruding a viscous aqueous solution onto a flexible web traveling at a linear speed of at least 150 feet per minute and 1 to 200 times faster than the linear speed of extrusion of the liquid, in the substantial absence of non-condensable gases, but in the presence of added readily condensable vapors of inert, water-soluble liquids having a boiling point of not greater than 230° F. at atmospheric pressure, passing the coated web at the same rate through a heated drying zone for 2 to 15 seconds, said zone being maintained at a pressure of 5 to 192 mm. of mercury, and the coated layer being at a temperature of 34° F. to 150° F. during its passage through said drying zone.

The novel processes of this invention in one of its broader aspects comprises extruding a viscous aqueous dispersion of silver halides in a water-permeable colloid having a viscosity of 2,000 to 100,000 and preferably 3,000 to 60,000 centipoises and a solids content of 20% to 65%, through a narrow, rectangular slot orifice onto a moving web of film or paper traveling at a speed of at least 150 feet per minute and at a linear speed the same or preferably faster than that at which the dispersion is extruded so that the extruded layer of dispersion is drawn down 1 to 200 times in thickness, at a reduced pressure, in the substantial absence of non-condensable vapors but in the presence of added water vapor at a pressure of 20 to 190 mm. and preferably 30 to 130 mm. of mercury and temperature of 75° F. to 150° F. and preferably 85° F. to 135° F., passing the coated film into a sealed drying chamber maintained at a total pressure from 5 to 35 mm. and preferably 15 to 25 mm. of mercury and where the film receives heat during which time the water is evaporated at approximately the boiling point of water corresponding to the vacuum maintained. The film temperature in the drying chamber will thus be between 34° F. and 90° F. and the emulsion will be dry after 2 to 15 seconds. The dry film leaves the drying chamber through suitable sealing mechanism and is then passed through a suitable windup station for storage and use or into a slitting and cutting mechanism where it is made into rolls of smaller width and length or sheets.

The lips of the rectangular slot orifice are placed about 0.002 to 0.030 inch apart and they are disposed about  $\frac{1}{16}$  to  $\frac{3}{16}$  inch above the surface of the web to be coated. The angle between the web and the center line of the extrusion lips should be from 0 degree to 60 degrees. Since the coating point is generally above a supporting roller of small diameter or curved bar of small radius the angle is measured from the tangent perpendicular to the axis

of such roller or bar at the point of contact of the extruded layer of dispersion.

In carrying out the process the coating chamber is provided with suitable sealing means at the point of entrance and at the point of exit of the web from the drying chamber. Also in its movement from the coating chamber to the drying chamber the web is conducted through a restricted opening so that a differential pressure can be maintained between the coating zone and drying zone, respectively.

The total pressure in the coating zone should be high enough to prevent the water and any water-soluble solvents in the aqueous dispersion being coated from boiling at the coating temperature which, with photographic gelatin emulsions, is usually about 90° F. to 110° F.

Air is purged from the coating zone before the coating operation commences by introducing a current of water vapor, e. g., saturated steam while evacuating the two zones by means of a vacuum pump or aspirator. Water vapor is introduced into the coating zone continuously during the coating operation and the added water vapor and any air which leaks into the system and any water or volatile solvents which evaporate from the emulsion are drawn off by means of a vacuum pump or aspirator.

When the aqueous coating solution contains a water-soluble solvent which has a relatively high vapor pressure, such as methyl alcohol, ethyl alcohol, and acetone, vapors of such solvents and/or water can be added to the coating zone.

Referring now to the accompanying drawings which constitute part of this specification,

Fig. 1 is a schematic, sectional view in elevation of one type of vacuum coater and dryer of this invention,

Fig. 2 is a schematic, sectional view in elevation of an alternative type vacuum coater and dryer of this invention, and

Fig. 3 is a perspective view with parts in section of the coating support roller and vapor induction tube.

The coating and drying apparatus shown in Fig. 1 of the drawings consists of an enclosed chamber 1 which is provided with an eduction pipe 2. The chamber is divided into two zones, a coating zone and a drying zone. A continuous web of photographic film base or paper from a source not shown passes through one wall of the chamber into the coating zone. This wall is provided with two hard surfaced (e. g. metal) rollers 3 which have resilient sealing means at their ends. A horizontal resilient roller 4 presses against the surface of horizontal rollers 3 and when the web is introduced between one of the rollers 3 and resilient roller 4, the admission of any significant amount of air into the coating chamber is prevented. The web passes in a horizontal plane over horizontally disposed roller 5 then downwardly under horizontal roller 6, then upwardly over horizontal coating support roller 7, then downwardly around a relatively large drum 8, which can be provided with means for regulating its temperature. The film then passes upwardly into the drying chamber. The coating chamber is separated from the drying chamber by means of an L-shaped baffle 9 which is provided at its ends with suitable resilient sealing means 10 which contact with the hard surface sealing roller 3 and another horizontally disposed hard surface sealing roller 11 between the surface of which and the surface of the drum 8 there is disposed another horizontally mounted resilient sealing roller 12.

The outer wall of the chamber 1 is curved and spaced a slight distance from the surface of the drum, thus acting as a baffle and providing a means of maintaining a pressure difference between the coating zone and the drying zone. Above the web supporting roller 7 there is disposed an extrusion hopper 13 which is provided with a narrow slot orifice for extruding the viscous aqueous silver halide dispersion onto the surface of the web. This extrusion hopper is similar to that described more fully below in the apparatus of Fig. 2 being shown in detail in Fig. 3.

The emulsion is fed into the hopper at a constant rate by means of a metering pump. It preferably is first passed through a heat exchanger which maintains the temperature uniform. The hopper may also be provided with temperature regulating means.

A horizontally disposed vapor tube 14 is placed adjacent to the coating support roller 7 so that solvent vapor or other condensable vapor can be introduced into the coating zone near the coating point. The absolute pressure in the coating zone is regulated by the amount of condensable vapor added.

The web W after leaving the coating chamber passes upwardly then over a horizontally disposed guide roller 15 which is journaled in bearings on a frame which can be moved upwardly or downwardly in the drying chamber to vary the length of film between heating elements (described below). The web then passes downwardly under a horizontal guide roller 16 then laterally between hard surface sealing roller 17 and resilient sealing roller 18, which in turn, presses against another horizontal hard surface sealing roller 17 which has a construction similar to roller 3. The upper end of the drying chamber is provided with heating platens 19 which are provided with suitable means for heating them to an elevated temperature, e. g., 300° F. to 1000° F. These platens may contain electrical resistance elements (e. g., infra-red heating platens) or may be provided with tubes for circulating a heat exchange fluid. Between the heating platens and the walls of the chamber, there is provided suitable insulation 20. It may be composed of any suitable insulation such as refractory insulating brick or aluminum foil. An inspection window 21 is provided in the wall of the chamber opposite the coating point.

In a practical apparatus of the type schematically shown in Fig. 1, the drum may be 2 to 4 feet in diameter and the drying zone 8 to 20 feet in height. The remaining rollers may have diameters proportional, as shown in the drawing, to such drum diameters.

The coating and drying apparatus shown in Fig. 2 of the drawings consists of a U-shaped chamber 31 which has a lateral eduction duct for vapor removal in the upper part of the chamber 32. There are disposed in the upper wall of the chamber horizontal hard-surface sealing rollers 33 and intermediate resilient sealing roller 34. Web W passes between the circumferential surfaces of the resilient sealing roll and the hard-surface sealing roll then downwardly under guiding roller 35, then upwardly over coating support roller 36, then downwardly and upwardly around drum 37 for the major portion of its diameter then under guiding roller 38 and upwardly between hard surface sealing roller 39 and resilient sealing roller 40, which in turn, is pressed against an additional hard-surface sealing roller 39. Each of the sealing rollers 33, 34, 39, and 40 are journaled in suitable bearings mounted on the frame for the chamber 31. Their ends and one face are provided with resilient sealing means to prevent the free ingress of air between the atmosphere and the chamber. Sealing means 33' and 39' are provided in the walls of the chamber to press against the peripheral surfaces of rollers 33 and 39, respectively.

A horizontal resilient sealing roller 41 is placed between the surface of drum 37 and one of the sealing rollers 39 or 33 (as shown) in order to separate the coating zone from the drying zone of the chamber. The lower curved wall of chamber 31 is U-shaped and, in general, follows the contour of the drum. It is maintained close to the drum, for example, about  $\frac{1}{8}$  of an inch therefrom from the point where the web passes onto the drum for a substantial distance so as to form a narrow confining passage for the web. This narrow passage, with sealing roller 41, serves to separate the coating chamber from the drying chamber so that the zones can be separately heated or exhausted to different temperatures and pressures.

In the lower portion of the chamber the lower U-shaped wall of the chamber 31 is spaced from the surface of the drum in order to form a U-shaped drying zone 42. Curved heating platens 42' are placed in this chamber and may be fastened to the walls by any suitable means. These heating elements can be electrically heated platens or platens heated by means of tubes through which a heat-regulating fluid is circulated. The upper part of chamber 31 opposite the coating zone that has the eduction opening 32, which is preferably a rectangular or circular tube, communicates with an aspirator expansion chamber 43. High pressure steam is passed through aspirator tube 44 which passes into the aspirator expansion chamber and withdraws vapors from the coating and heating zone. The aspirator expansion chamber communicates with a cooling chamber 45 which is provided with suitable horizontal staggered baffles 46. Water is passed through pipe 47 into the cooling chamber where it passes downwardly over the baffles and absorbs the vapors passing into the chamber. Any remaining vapors pass upwardly through pipe 48 which connects with aspirator 49 and high pressure steam is injected into this aspirator by a suitable tube 50. The lower end of the cooling chamber is provided with an outlet tube 51 which communicates with a pump 52.

Above coating support roller 36 there is provided an extrusion hopper 54, details of which are more fully described below with regard to Fig. 3. Adjacent to the extrusion hopper there is provided a vapor tube 59 for the introduction of water vapor or other condensable vapor near the coating point. In the wall opposite the extrusion hopper there is provided a window 53 so that the point of coating can be observed. The emulsion is fed into the hopper at a constant rate by means of a metering pump. It preferably is first passed through a heat exchanger which maintains the temperature uniform. The hopper is also provided with temperature regulating means.

The drum in the type of apparatus shown in Fig. 2 may be 8 to 20 feet in diameter and the other rollers proportional in size to the drum, as indicated in the drawing.

The apparatus shown in Fig. 2 is not limited to an aspirator for removing vapors from the drying zone as a vacuum pump or other suitable vacuum producing means can be connected to the eduction opening 32. Other means of condensing the vapors may be employed such as tubular heat exchangers.

Referring now to Fig. 3, the induction hopper 54 has a horizontal throat 55 which connects with a source of viscous aqueous solution, e. g., an aqueous silver halide dispersion. The throat communicates with lips 56 which are spaced a short distance apart, e. g., 0.002 inch to 0.030 inch. One or both of these lips may be made adjustable so that the width of the opening between the lips can be closely adjusted. It may be fastened to the hopper by means of screws 57. The hopper is also provided with channels 58 through which a heat exchanging fluid can be circulated to control the temperature of the hopper. The lips of the hopper should be accurately machined and highly finished and they should be as nearly parallel as possible so as to result in a uniform thickness of the extruded emulsion. The upper surface of the bottom hopper lip is placed about  $\frac{1}{16}$  to  $\frac{3}{16}$  inch from the surface of the web.

Vapor tube 59 is placed adjacent to the hopper so that water vapor or other condensable vapor is projected under the hopper between the web and the extruded layer of silver halide dispersion.

Suitable sealing means for the ends of the rolls 3, 4, 12, 17, 18, 33, 34, 39, and 41, etc. for seals 10, 33' and 39' of the two above-described types of apparatus, are described in Minton U. S. Patent No. 1,633,121. This patent also discloses suitable sealed journalled bearings which

are useful for mounting the sealing rolls in the apparatus of the invention.

Various gears, belts or chains and attendant mechanisms which are connected to a suitable source or sources of power can be used to drive the drum and coating roller. They can be synchronized with each other and with suitable web windup and feed devices. Rapid change mechanisms, etc., to permit substituting a new roll of web and splicing it to the end of the old roll, can be supplied to make the operation continuous over long periods of time.

The heating elements or platens used in the above apparatus should be constructed so that they do not emit any substantial amounts of actinic light which would expose and thus affect the coated layer deleteriously. These platens may be electrically heated and should provide uniform concentration of radiant energy over the entire surface exposed.

An important feature of each of the above apparatus resides in the use of a coating support roller of relatively small diameter, e. g., from  $\frac{1}{4}$ " to  $\frac{3}{4}$ ". The use of such small diameter support rolls is unique and gives surprising and unexpected results. Thus, it has been found that with rollers of these small diameters more than a four-fold increase in coating speed can be attained than with coating support rollers with twice the diameter or more. For example, in test measurements with one viscosity of silver halide emulsion coating, speeds of 96 to 129 feet per minute were attained with a roller of  $\frac{1}{4}$ " in diameter, whereas coating speeds of 21 to 30 feet per minute were attained with a roller of  $1\frac{1}{2}$ " in diameter. The smaller diameter coating roller enables one to use a wider angle of nip between the locus of the path of the extruded film and the tangent to the roller surface. A stationary curved coating bar of equally small radius can be used in place of the roller if desired. It has been found that a wider angle of nip admits of faster coating speeds and substantially eliminates entrapment of vapor between the emulsion and base.

The operation of the above combined coating and drying apparatus and the above processes will be more fully described in the following examples.

#### Example I

An aqueous gelatino silver iodobromide emulsion of the X-ray type (50% by weight solids content) is extruded through an emulsion hopper onto a thin gelatin substratum on a cellulose acetate film base having a thickness of about 8 mils and a width of about 45", to a coating weight of about 103 milligrams of silver halide per square decimeter, in an apparatus of the type shown in Fig. 1 of the drawing. The air is removed from the apparatus by introducing a jet of steam while evacuating the drying chamber to a pressure of 18 to 40 mm. of mercury. The coating zone is maintained at a temperature of 95° F. to 110° F. and saturated steam is introduced into the coating zone to maintain a partial pressure of water of 42 to 66 mm. of mercury. The lips of the coating hopper are spaced 0.005 to 0.010 inch apart and they are disposed about  $\frac{1}{8}$  inch from the point of contact with the web on the coating support roller which has a diameter of  $\frac{3}{4}$  inch. The emulsion is extruded at the rate of 40-80 feet per minute and the web is moved past the coating point at the rate of 400 feet per minute. The infra-red heating platens in the drying zone are maintained at a temperature of about 1000° F. The length of the heating platens is about 10 feet and any given point on the film is maintained in the drying zone about three seconds. As the coated film emerges from the coating and drying apparatus, it is found to be smooth, firm and of uniform photographic quality, with properties similar to a film dried in air in the conventional manner.

## Example II

A gelatino silver iodobromide emulsion of the type described in Example I is prepared and coated onto a film element of the type described in that example but in an apparatus of the type shown in Fig. 2 of the drawing. The air is first removed from the apparatus by aspirators which maintain a vapor pressure of 6 to 10 mm. of mercury in the drying chamber. Steam is admitted to the coating chamber at a rate to maintain a pressure of 60 to 70 mm. in such coating chamber. The drum is approximately 10 feet in diameter and heated to a temperature of 105° F. to 110° F. and the heating platens are heated to a temperature of 900° F. to 1000° F. The coated film remains in the drying chamber for about three to four seconds. As it emerges from the drying chamber, it is found to be smooth, firm and of uniform photographic quality. The film has properties similar to a film dried in air in the conventional manner.

The apparatus described above is not limited to the use of electric means for heating the platens nor to the passage of a heated exchange fluid through ducts or tubes, as induction heating may be used. The drum can be heated by means of induction coils or by passing a heat exchange fluid through channels or ducts near its surface or by other suitable means.

In place of the extrusion hoppers, there can be substituted a pair of closely fitting rollers. The viscous solution is fed into the nip of such rollers and forced between them to form a film.

The invention is, of course, not limited to the coating of film and paper with aqueous gelatin silver halide emulsions but is useful in coating aqueous silver halide dispersions in other water-permeable colloids as described above. Thus, it can be used in the coating of aqueous ethanol solutions of polyvinyl acetal color formers of the type described in Jennings et al. U. S. Patent 2,397,864 and Blanchard U. S. Patent 2,551,091.

The invention is useful in preparing multilayer photographic film elements including multicolor films both positive and negative, printing papers, double-coated X-ray films, motion picture films, portrait films, and papers, etc. It is not only useful in coating the light-sensitive silver halide colloid layers but can be used in coating light-filter layers, and antihalation layers containing dyes and pigments which absorb the desired wavelengths of light, as well as antiabrasion layers and sublayers from aqueous solutions, including aqueous ethanol solutions. In these layers gelatin or the other colloids described above may constitute the film-forming binding agent. The coating solutions may have a solids content of 20% to 65%.

An advantage of the invention resides in the fact that photographic film and paper may be coated and dried in an extremely short time as compared with prior art methods. Thus, the film can be dried in three to five seconds at relatively low temperatures. The high drying rate admits of considerable savings in labor and in fixed overhead for the photographic manufacturer. The apparatus has the advantage that it is very compact and requires only a fraction of the building space usually required for the convection type of dryer.

The elimination of the convection drying chambers and attended equipment results in considerable power savings which are normally required for refrigerating large quantities of air, operating large blowers, reheating the refrigerated air, recovering solvents, etc.

The process of the present invention requires relatively small quantities of added vapor, e. g., steam. Relatively small amounts of electric power, steam and other utilities are required for the operation of the vacuum coating and drying apparatus of this invention as compared with the convection type coater and dryer of equivalent capacity.

The invention has the further advantage that dust particles are not likely to come into contact with the wet

coating material. Also the extremely short travel of the wet emulsion within a sealed chamber makes dust collection extremely unlikely.

The problem of static generation within the dryer is eliminated due to the fact that gases are more easily ionized at low pressures. Thus, it has been found that static charges, which might harm the sensitized emulsion, do not build up within the evacuated dryer.

Film dried in vacuum at temperatures below 90° F. has a low surface resistivity ( $5 \times 10^{12}$ ) so that it will not be abnormally susceptible to static troubles later on in its manufacture or use. Film dried in so short a time by any other method would have a high surface resistivity and would be likely to pick up static marks in handling subsequent to the drying operations. Still other advantages will be apparent from the above description of the invention.

What is claimed is:

1. The process which comprises extruding in a coating zone within a chamber a viscous aqueous solution onto a moving flexible web traveling at a linear speed of at least 150 feet per minute and 1 to 200 times faster than the linear speed of extrusion of the dispersion, in the substantial absence of non-condensable gases, but in the presence of added readily condensable vapors of inert, water-soluble liquids having a boiling point of not greater than 230° F. at atmospheric pressure, passing the coated web at the same rate of speed through a heated drying zone within said chamber for 2 to 15 seconds, said drying zone being maintained at a pressure of 5 to 192 mm. of mercury and the coated layer being at a temperature of 34° F. to 150° F. during the drying stage.
2. The process which comprises extruding in a coating zone within a chamber a viscous aqueous solution containing a water-permeable colloid onto a moving flexible web traveling at a linear speed of at least 150 feet per minute and 1 to 200 times faster than the linear speed of extrusion of the dispersion, in the substantial absence of non-condensable gases, but in the presence of added readily condensable vapors of inert, water-soluble liquids having a boiling point of not greater than 230° F. at atmospheric pressure, passing the coated web at the same rate of speed through a heated drying zone within said chamber for 2 to 15 seconds, said drying zone being maintained at a pressure of 5 to 35 mm. of mercury and the coated layer being at a temperature of 34° F. to 90° F. during the drying stages.

3. The process which comprises forming a viscous aqueous dispersion of silver halides in a water-permeable colloid in the form of a layer 0.002 to 0.030 inch in thickness, in a zone within a chamber, said zone being maintained at a pressure from 20 to 190 mm. of mercury and a temperature of 75° F. to 150° F., passing said layer onto a moving flexible web traveling at a linear speed of at least 150 feet per minute and 1 to 200 times faster than the linear speed of extrusion of the dispersion, in the substantial absence of non-condensable gases, but in the presence of added readily condensable vapors of inert, water-soluble liquids having a boiling point of not greater than 230° F. at atmospheric pressure, passing the coated web at the same rate of speed through a heated drying zone within said chamber for 2 to 15 seconds, said drying zone being maintained at a pressure of 5 to 35 mm. of mercury and the coated layer being at a temperature of 34° F. to 90° F. during the drying stages.

4. The process which comprises extruding a viscous aqueous dispersion of silver halides in a water-permeable colloid having a viscosity of 2,000 to 100,000 centipoises and a solids content of 20% to 65%, in the form of a layer 0.002 inch to 0.030 inch in thickness, into a zone within a chamber, said zone being maintained at a pressure from 20 to 190 mm. of mercury and a temperature of 75° F. to 150° F., and onto a moving flexible web traveling at a linear speed of at least 200 feet per minute and 1 to 200 times faster than the linear speed of extru-

sion of the dispersion, in the substantial absence of non-condensable gases, but in the presence of added readily condensable vapors of an inert, water-soluble liquid having a boiling point of not greater than 230° F. at atmospheric pressure, passing the coated web at the same rate of speed through a drying zone within said chamber where the required amount of heat is supplied in a period of 2 to 15 seconds and where the pressure is maintained at 5 to 35 mm. of mercury which in turn results in an emulsion temperature of 34° F. to 90° F. during the drying stage.

5. The process which comprises extruding a viscous aqueous dispersion of silver halides in a water-permeable colloid having a viscosity of 2,000 to 100,000 centipoises and a solids content of 20% to 65%, in the form of a layer 0.002 inch to 0.030 inch in thickness, into a zone within a chamber, said zone being maintained at a pressure from 20 to 190 mm. of mercury and a temperature of 75° F. to 150° F., and onto a moving flexible web traveling at a linear speed of at least 150 feet per minute and 1 to 200 times faster than the linear speed of extrusion of the dispersion, in the substantial absence of non-condensable gases, but in the presence of added water vapor, passing the coated web at the same rate of speed through a drying zone within said chamber where the required amount of heat is supplied in 2 to 15 seconds and where the pressure is maintained at 5 to 35 mm. of mercury which in turn results in an emulsion temperature of 34° F. to 90° F. during the drying cycle.

6. A process as set forth in claim 5 wherein said colloid is gelatin.

7. A process as set forth in claim 6 wherein the water vapor is added in an amount sufficient to keep the water

in the aqueous dispersion from boiling at the coating temperature.

5 8. A process as set forth in claim 5 wherein said colloid is a hydroxyl polymer containing a large number of recurring intralinear —CH<sub>2</sub>CHOH— groups.

10 9. The process which comprises extruding an aqueous dispersion of light-sensitive silver halides in gelatin having a viscosity of 3,000 to 60,000 centipoises and a solids content of 20% to 65% by weight in the form of a layer 0.002 inch to 0.030 inch in thickness, into a zone within a chamber, said zone being maintained at a pressure from 30 to 130 mm. of mercury and a temperature of 85° F. to 135° F., onto a thin flexible film traveling at a linear speed of 350 to 500 feet per minute and 1 to 200 times 15 faster than the linear speed of extrusion of the dispersion, in the substantial absence of non-condensable gases, but in the presence of added water vapor, passing the coated web at the same rate of speed through a heated drying zone within said chamber for 2 to 15 seconds and where 20 the pressure is maintained at 5 to 35 mm. of mercury and the emulsion is at a temperature of 34° F. to 90° F.

References Cited in the file of this patent

UNITED STATES PATENTS

|    |           |              |       |                |
|----|-----------|--------------|-------|----------------|
| 25 | 1,493,000 | Morse        | ----- | May 6, 1924    |
|    | 1,735,689 | Maas         | ----- | Nov. 12, 1929  |
|    | 1,861,918 | Hickman      | ----- | June 7, 1932   |
|    | 2,175,125 | Mack et al.  | ----- | Oct. 3, 1939   |
|    | 2,469,633 | Corson       | ----- | May 10, 1949   |
| 30 | 2,519,728 | Alexander    | ----- | Aug. 22, 1950  |
|    | 2,610,937 | Frink et al. | ----- | Sept. 16, 1952 |
|    | 2,681,294 | Beguin       | ----- | June 15, 1954  |